

Jan. 2, 1934.

C. R. KUZELL

1,941,606

METALLURGICAL APPARATUS

Filed Nov. 19, 1929

Fig. 1



Fig. 2



INVENTOR

Charles R. Kuzell

BY

Tennie, Davis, Marvin & Edmonds  
HIS ATTORNEYS

## UNITED STATES PATENT OFFICE

1,941,606

## METALLURGICAL APPARATUS

Charles R. Kuzell, Clarkdale, Ariz., assignor to  
 United Verde Copper Company, Clarkdale,  
 Ariz., a corporation of Delaware

Application November 19, 1929  
 Serial No. 408,247

13 Claims. (Cl. 266—43)

This invention relates to metallurgical apparatus and has for an object the provision of an improved receptacle for receiving molten baths for treatment. More particularly, the invention 5 contemplates the provision of an improved receptacle having an improved heat refractory and molten bath resistant lining. The invention further contemplates the provision of an improved refractory lining material and an improved method 10 of lining molten bath receptacles with basic materials. In one of its more limited aspects, the invention contemplates the provision of an improved basic lined copper converter.

In processes involving the treatment of molten baths at high temperatures, it is customary 15 to employ receptacles for the baths which comprise sheet metal shells lined with refractory materials. The nature of the refractory material employed is determined by the nature of the 20 process and the composition or character of the bath. Thus, in some instances, acid refractories such as silica are employed, while in other instances, basic refractories such as magnesite are employed. The form in which the refractory 25 material is applied to the inner surface of the receptacle depends largely upon the character of the material and to some extent upon the nature of the process to be carried out. The character of a refractory material may be such that it may 30 be employed in providing a monolithic lining for use in a particular process, or its character may be such that it can only be successfully employed in the form of bricks which have been subjected to high temperatures and/or pressures. Frequent 35 replacement of linings is necessary in many cases because of rapid destruction and disintegration resulting from high temperatures, corrosion and other causes. Monolithic linings, as a general rule, may be provided at a lower cost than brick 40 linings, and it is therefore advisable when possible to use refractory material which is capable of forming satisfactory monolithic linings or to so form a monolithic lining from ordinarily unsuitable material that satisfactory service may be 45 obtained.

According to some present practices, molten bath receptacles employed in processes requiring the use of basic linings are lined with bricks. It is generally believed that such linings must be 50 formed of bricks of properly heat treated material and that a monolithic lining cannot be successfully employed. The use of basic materials in brick form is, in some instances, satisfactory from the operating standpoint, but patching 55 of brick linings and replacement of burned out

portions is usually a difficult and costly procedure. In replacing a portion of a brick lining, it is generally necessary to remove a considerable portion of the lining adjacent the burned out portion to provide smooth, flat contact surfaces. 60 This involves the destruction and removal of a considerable amount of substantially unimpaired lining and enforced idleness of the receptacle for a relatively long period. Furthermore, bricks are relatively costly and, in some instances, the lining replacement cost constitutes a major operating cost. 65

Various factors contribute to the destruction and disintegration of linings. Thus, in copper smelting operations, basic converter linings are 70 injured by the heat of the charge, by changes in temperature, and by the corrosive action of the slag and matte. The action of an improper slag is probably the more harmful, and the character of the slag must therefore be carefully controlled. Slags containing large amounts of silica attack basic linings, and, consequently, slags containing relatively small amounts of silica are used in copper converting operations employing converters lined with expensive basic 80 brick such, for example, as magnesite brick in order to avoid destruction of the lining. It is probable that the corrosive effect of high-silica slags as compared with low-silica slags may be attributed largely to the fact that in the case of 85 high-silica slags little or no magnetite is formed and deposited on the lining while low-silica slags are conducive to the production of magnetite which is deposited on the linings and provides protective coatings therefor. 90

While the use of a slag having a low silica content prolongs the life of a converter lining, such slags also produce certain harmful effects. Low-silica slags retain more copper than high-silica slags, the amount of copper carried by the 95 slag being inversely proportional to the amount of silica contained therein. Considerable difficulty is experienced in handling low-silica slags in ladles and in introducing such slags into retreatment furnaces. Retreatment of low-silica 100 slags also involves some difficulties. It is difficult to extract copper from such slags, and there is a tendency for magnetite contained therein to separate out and build accretions on the hearth of the retreatment furnace. 105

The present invention contemplates the provision of a method of lining molten bath receptacles to obtain monolithic linings which are satisfactory in service and which are less costly and more easily repaired than brick linings. 110

The invention further contemplates the provision of a copper converter provided with a basic lining which may be replaced at a cost which will permit the use of relatively high-silica slag to avoid copper losses and to minimize handling and retreatment difficulties.

According to the present invention, granulated basic refractory material is mixed with a suitable binder in the wet state and rammed or tamped into place between the receptacle wall and a suitable form to provide a wall of proper thickness. When the lining material has been rammed or tamped into place, the form is removed and the wet lining is subjected to heat at a low temperature for a sufficiently long period to drive off the major portion of the water contained therein. The lining is subsequently heated until it reaches a temperature approximating that to which it will be subjected in service to a temperature which is high enough that the charging of a bath of normal temperature will not cause material damage. It is unnecessary to bring the entire lining up to the maximum temperature. Good results can be obtained if only that portion of the lining immediately adjacent the inner surface is thus heated.

In order that the best results may be obtained in forming the refractory lining material of the invention, it is important that the particle sizes be carefully proportioned. The most satisfactory material comprises a mixture of relatively fine particles and relatively coarse particles. The coarse particles should form the major portion of the mixture. The fine particles should be sufficiently small to form a compact mass which is substantially impervious to, or capable of affording satisfactory resistance to penetration by, the molten mineral bath in conjunction with which the lining is to be used. The relative amounts of fine and coarse material to be used in each case will depend upon the character and sizes of the coarse grains. Sufficient fine material to fill the voids between the coarse particles should be used. It is desirable, though not necessary, to provide just sufficient fine material to fill the voids and permit at least one point of contact of each coarse particle with every adjacent coarse particle.

The fine material may consist substantially entirely of particles ranging from substantially colloidal particles to 80-mesh, and the coarse material may consist substantially entirely of particles ranging from 20-mesh to one-half inch or larger. In general, it is advisable to use mixtures of which thirteen to twenty per cent of the particles are sufficiently small to pass an 80-mesh screen. A large proportion of the remaining particles should be too large to pass a 20-mesh screen. About eighty per cent of the minus 80-mesh material should pass a 200-mesh screen. The proportion of particles between 20-mesh and 80-mesh in size should be minimized. In fact, it is desirable to eliminate such sized particles. While any suitable mixture of grain sizes may be used, the best results may be obtained when no intermediate sizes are used and when thirteen to twenty per cent of the particles pass an 80-mesh screen and the remaining particles are too large to pass a 20-mesh screen. Material in which ten to fifteen per cent of the particles are too large to pass a 3-mesh screen is very satisfactory.

Particle sizes have been given in terms of

the Tyler series. Percentages by weight are given throughout the specification.

The mixtures of particles of different sizes may be formed in any desired manner. A number of different sizes may be separately formed and classified and subsequently mixed in the proper proportions, or crushing and grinding may be so conducted that very coarse material may be reduced to provide a mixture containing approximately the correct sizes and proportions in a single operation. The composition of the resulting mixture may be corrected by additions of separately classified particles of the proper sizes. Satisfactory coarse and fine products may be obtained by subjecting the raw or initial materials to types of treatment designed to produce particles having maximum sizes corresponding to the maximum sizes desired. In each case the grinding or crushing operations utilized will produce a mixture containing the maximum and minimum sizes as well as a variety of intermediate sizes. If the resulting products are not satisfactory separate additions and/or removal of particles of particular sizes may be made.

Any suitable solid or liquid substance may be used as a bonding agent. The binder may comprise a plastic mass of finely divided solid particles. When a binder comprising solid particles is used, the binder may provide a portion of the fine material required for the lining mixture.

The binder should be selected to avoid the incorporation of large amounts of fluxing materials in the lining. The following binders have been found to be satisfactory when used with granular magnesite in the amounts by weight noted:

|                                                              | Percent   |
|--------------------------------------------------------------|-----------|
| Fireclay                                                     | 2 - 5     |
| Bauxite                                                      | 2 - 10    |
| A mixture containing bauxite 3 parts<br>and fireclay 2 parts | 2 - 10    |
| Molasses                                                     | 0.5 - 5.0 |

The lining mixture should contain sufficient water or other fluid that a plastic mass capable of being tamped to form a dense structure is provided. A water or fluid content of about 3 to 5% by weight is ordinarily satisfactory.

Owing to the fact that in crushing or grinding refractory materials an infinite variety of particle shapes may be produced, it is substantially impossible to predict that any mixture of particles of different sizes will result in the production of a perfect lining. Mixtures of particles within the size limits hereinbefore set forth produce satisfactory linings, and the most satisfactory mixture for any particular material or for any particular purpose may be determined readily by means of a few simple tests. For example, small amounts of several different mixtures may be formed into bricks which may be subjected to conditions similar to those to which the lining will be subjected, and a comparison of the effects on the different bricks will indicate the mixture which is the more suitable.

Magnesite linings formed in accordance with the method of the present invention are particularly suitable for use in copper converters, and when so used give satisfactory service at a lower cost than brick linings of similar materials. California magnesite may be used advantageously. Two commercial forms of magnesite, dead burned magnesite and periclase, have been found to be satisfactory for forming linings in accordance with the method of the invention. A number of magnesite linings which served satisfac-

torily in copper converters showed matte and slag penetration varying from about one-half inch to about one and three-quarter inches.

Linings of the invention have been successfully used in copper converters, twelve feet in diameter, of the type illustrated in the accompanying drawing, in which

Fig. 1 is a sectional side elevation of a well-known type of copper converter provided with a monolithic lining; and

Fig. 2 is a section taken substantially along line 2-2 of Fig. 1.

The converter comprises a substantially cylindrical receptacle having sheet metal side walls 10 and a sheet metal bottom wall 11. The side walls and bottom of the receptacle are provided with a monolithic lining 12. A tuyère pipe 13 extends through the side wall 10 and the lining 12 and provides means of communication between the interior of the receptacle and a source of supply of air under pressure (not shown). A layer or lining 17 of heat insulating bricks is disposed between the sheet metal side wall 10 and the monolithic lining and extends around the receptacle in the vicinity of the tuyère pipe. A substantially conical cap 14 provided with an opening 15 in its side wall and having a monolithic lining 16 is removably mounted on the receptacle.

When the converter is to be lined, the cap is removed to permit the insertion of forms. The bottom is first provided with a layer of a suitable refractory mixture of the desired thickness which is tamped to provide a dense structure. When the bottom has been lined, forms having substantially vertical walls are placed within the receptacle with their vertical walls spaced the proper distances from the vertical side walls of the receptacle. The lining mixture is then placed between the form and the side walls in successive horizontal layers of suitable thickness. Each layer is thoroughly tamped and packed before the next succeeding layer is added. The best results have been obtained when the material has been inserted in layers varying from three to seven inches in thickness. Layers of greater thickness are difficult to tamp properly and their use might result in segregation of the coarse particles. The insulating and protecting bricks are placed in position in layers periodically as the lining mixture is inserted. The tuyère pipes are inserted when the lining has been built to the proper height. The lining mixture is tamped and packed around the sides and above the tuyère pipes. During the tamping, bars or heavy pipes may be inserted within the tuyère pipes to prevent distortion. The force used in tamping need only be sufficient to insure thorough packing and the production of a dense mass.

The cap is separately lined while inverted. The cap may be lined with the lining mixture of the invention or any other suitable refractory. The caps are not subjected to excessive wear and the cost of their linings is not of great importance. The joint between the cap lining and the shell lining when the cap is attached may be plastered with the lining mixture of the invention or any suitable plastic mass of refractory material.

When the lining has been completed a slow wood fire is started in the receptacle and heating is conducted in this manner until the lining has been well dried. This requires from about eight to forty-eight hours depending probably upon the heat generated, the thickness of the lining, and the amount of moisture in the lining. When

the lining has been dried satisfactorily in this manner, it is heated by means of a hot oil fire for a sufficiently long period to raise the temperature of the inner surface portion thereof to about 2000° F. This heating may be continued over a period of from eight hours to several days.

The converter should be put in service before any considerable drop in the temperature of the lining takes place. The usual procedure with respect to copper converters may be followed in putting the converter into service. A coating of magnetite may be provided or not as desired. Better service will be obtained if copper is not made within forty-eight hours after the converter is put into operation.

The monolithic linings of the present invention are not only satisfactory in service when new, but they may also be quickly and cheaply repaired when portions thereof are damaged. In patching a damaged monolithic lining it is only necessary to cut away a sufficient amount of the old lining to provide a rough surface for bonding purposes and apply a suitable amount of the lining mixture to build the damaged portion to the required thickness.

It is advisable to dry and burn patches in the same manner as new linings prior to putting the receptacles back in service.

Linings formed in accordance with the present invention are considerably cheaper than linings formed from refractory bricks according to the heretofore customary practices. Granular material can be obtained more cheaply than bricks at any desired location. The linings of the invention can be installed at a lower cost than brick linings. The installation of brick linings requires highly skilled labor while the installation of the linings of the invention may be made by relatively cheap common labor.

The relatively lower cost of monolithic basic linings of the invention permits the use of a more siliceous slag in copper converters even though the siliceous slag attacks the lining. The use of a siliceous slag is not only advantageous because of the lesser amount of copper carried thereby, but it is more advantageous because a relatively high-silica slag is easier to handle in ladles, easier to introduce into retreatment furnaces, and retreatment is more complete not only with respect to the copper extracted but also with respect to minimizing the segregation of the more or less infusible and refractory magnetite which, in the case of less siliceous converter slags, separates out in the retreatment furnaces and builds accretions on the hearth. Thus, the use of the linings of the invention permits not only saving in lining costs but a saving in the cost of retreatment and a higher recovery of copper as well.

I claim:

1. Refractory lining material comprising a mixture of granular magnesite and a solid binder in which about thirteen to twenty per cent of the particles are minus 80-mesh and about eighty per cent of the minus 80-mesh particles are minus 200-mesh.

2. Refractory lining material comprising a bonded mixture of granular magnesite and a solid binder in which about eighty to eighty-seven per cent of the particles are plus 80-mesh and in which about eighty per cent of the remaining particles are minus 200-mesh.

3. A molten bath receptacle having a monolithic refractory lining in which about thirteen to twenty percent of the bonded particles are minus 80-mesh, about eighty to eighty-seven percent

are plus 20-mesh and about ten to fifteen percent are plus 3-mesh, and in which about eighty percent of the minus 80-mesh particles are minus 200-mesh.

5. Lining material comprising a mixture of granular magnesite and a binder in which about thirteen to twenty percent of the particles are minus 80-mesh and the major portion of the remaining particles are plus 20-mesh, the binder being present in the mixture in an amount equal to about 0.5 to 10.0 percent by weight of the mixture.

10. Lining material comprising a mixture of granular magnesite and fireclay in which about thirteen to twenty percent of the particles are minus 80-mesh and the major portion of the remaining particles are plus 20-mesh, the fireclay being present in the mixture in an amount equal to about 2.0 to 5.0 percent by weight of the mixture.

15. Lining material comprising a mixture of granular magnesite and bauxite in which about thirteen to twenty percent of the particles are minus 80-mesh and the major portion of the remaining particles are plus 20-mesh, the bauxite being present in the mixture in an amount equal to about 2.0 to 10.0 percent by weight of the mixture.

20. Lining material comprising a mixture of granular magnesite and molasses in which about thirteen to twenty percent of the particles are minus 80-mesh and the major portion of the remaining particles are plus 20-mesh, the molasses being present in the mixture in an amount equal to about 0.5 to 5.0 percent by weight of the mixture.

25. A copper converter having a monolithic lining comprising magnesite and a binder and in which about thirteen to twenty percent of the bonded particles are minus 80-mesh, the remaining particles are plus 80-mesh, and about eighty percent of the minus 80-mesh particles are minus 200-mesh.

30. A molten bath receptacle having a monolithic lining made from a mixture comprising

magnesite and a binder in which about thirteen to twenty percent of the bonded particles are minus 80-mesh, the remaining particles are plus 80-mesh, and the major proportion of the minus 80-mesh particles are minus 200-mesh, the binder being present in the mixture in an amount equal to about 0.5 to 10.0 percent by weight of the mixture.

35. A molten bath receptacle having a monolithic lining made from a mixture comprising magnesite and a fireclay in which about thirteen to twenty percent of the bonded particles are minus 80-mesh, the remaining particles are plus 80-mesh, and the major proportion of the minus 80-mesh particles are minus 200-mesh, the fireclay being present in the mixture in an amount equal to about 2.0 to 5.0 percent by weight of the mixture.

40. A molten bath receptacle having a monolithic lining made from a mixture comprising magnesite and bauxite in which about thirteen to twenty percent of the bonded particles are minus 80-mesh, the remaining particles are plus 80-mesh, and the major proportion of the minus 80-mesh particles are minus 200-mesh, the bauxite being present in the mixture in an amount equal to about 2.0 to 10.0 percent by weight of the mixture.

45. A molten bath receptacle having a monolithic lining made from a mixture comprising magnesite and molasses in which about thirteen to twenty percent of the bonded particles are minus 80-mesh, the remaining particles are plus 80-mesh, and the major proportion of the minus 80-mesh particles are minus 200-mesh, the molasses being present in the mixture in an amount equal to about 0.5 to 5.0 percent by weight of the mixture.

50. Refractory lining material comprising a mixture of granular magnesite and a binder in which about thirteen to twenty percent of the particles are minus 80-mesh and the major proportion of the minus 80-mesh particles are minus 200-mesh.

CHARLES R. KUZELL. 120

50

126

55

130

60

135

65

140

70

145

75

150